

# UNITED STATES PATENT OFFICE.

CARL A. W. VOLLRATH, OF SHEBOYGAN, WISCONSIN, ASSIGNOR TO THE  
JACOB J. VOLLRATH MANUFACTURING COMPANY, OF SAME PLACE.

## PROCESS OF ENAMELING METAL SURFACES.

SPECIFICATION forming part of Letters Patent No. 415,485, dated November 19, 1889.

Application filed September 23, 1889. Serial No. 324,813. (No specimens.)

*To all whom it may concern:*

Be it known that I, CARL A. W. VOLLRATH, of Sheboygan, in the county of Sheboygan, and in the State of Wisconsin, have invented 5 certain new and useful Improvements in the Art of Enameling Metal Surfaces; and I do hereby declare that the following is a full, clear, and exact description thereof.

My invention relates to improvements in 10 the process of enameling metal surfaces, and will be fully set forth hereinafter and subsequently claimed.

In carrying out my process I proceed as follows: The iron or metal plates or other articles 15 to be enameled are first subjected to the ordinary pickling or scouring operations for the purpose of removing the scale and preparing the surface for the reception of the enameling composition.

20 I first prepare what I term the "ground mass" or "foundation-coating," the same consisting of a mixture of fifty parts of flint or quartz sand, thirty to sixty parts of borax, and five to ten parts of lime melted together 25 in a suitable crucible, and taken therefrom, cooled, and ground with water into a paste and distributed over the surface of the metallic article by pouring, dipping, or other convenient means, and then dried, and the article 30 so coated is then put in a suitable muffle or furnace and subjected to a temperature of about 1,000° Fahrenheit, which results in the production of a smooth glossy surface having a beautiful mottled appearance.

If desired, the "finishing-coating" (consisting of mixtures A and B) may be applied directly to the cleaned metallic articles; but 35 ordinarily I prefer to apply a foundation-coating, as first described; but in either event the object of my present invention is the production automatically upon metal surfaces of a mottled or pleasingly-speckled appearance 40 consequent, chiefly, upon the different degrees of fineness to which my mixture A and mixture B have been ground prior to mixing these two mixtures together.

Having thus described my invention, what I 45 claim as new, and desire to secure by Letters Patent, is—

50 1. In the art of enameling metal surfaces, the hereinbefore-named process, consisting of mixing and melting together the various 55 ingredients of an enameling composition, cooling the same, and grinding the resulting mass to a certain degree of fineness, then separately mixing and melting together similar ingredients with coloring-matter added there-

60 65 70 75 80 85 90 95 100

1. In the art of enameling metal surfaces, the hereinbefore-named process, consisting of mixing and melting together the various 95 ingredients of an enameling composition, cooling the same, and grinding the resulting mass to a certain degree of fineness, then separately mixing and melting together similar ingredients with coloring-matter added there-

- to, cooling the same, and grinding this resulting mass to a different degree of fineness from that to which the first mixture was reduced, then mixing together the two ground products in a moist condition of a paste-like consistency, applying this resulting product to the metal surfaces, and subjecting the goods thus coated to heat in a suitable muffle, substantially as set forth.
- 10 2. The hereinbefore-described art of automatically producing a mottled enamel upon metal surfaces, consisting in pickling or scouring the same to remove scale, applying a ground mass or foundation-coating thereto, and fixing it by subjecting the articles to heat in a suitable muffle, mixing and melting together two like mixtures of the various ingredients of an enameling composition in separate crucibles, one having coloring-matter added thereto, cooling the same, and grinding the two resulting masses to different de-

grees of fineness and with the finest ground in a moist condition, adding clay to the mass which is ground the finer of the two, and mixing the two ground masses together, in 25 the proportions of about one part of the coarse-ground mass to three parts of the fine-ground mass, to a paste-like consistency, applying the resulting product to the metal surfaces having the described foundation-coating, and subjecting the goods thus coated to heat in a suitable muffle, substantially as set forth.

In testimony that I claim the foregoing I have hereinunto set my hand, at Sheboygan, in 35 the county of Sheboygan and State of Wisconsin, in the presence of two witnesses.

CARL A. W. VOLLRATH.

Witnesses:

GUSTAV A. RIESS,  
FELIX BENFEY.